

Aug. 24, 1926.

1,597,010

K. BUBLA

PROCESS OF IMPREGNATING WOOD

Filed June 15, 1925



Inventor:  
Karl Bubla  
*[Signature]*  
Atty.

Patented Aug. 24, 1926.

1,597,010

# UNITED STATES PATENT OFFICE.

KARL BUBLA, OF PILSEN, CZECHOSLOVAKIA.

## PROCESS OF IMPREGNATING WOOD.

Application filed June 15, 1925, Serial No. 37,218, and in Czechoslovakia June 20, 1924.

My invention refers to the impregnating of wood, more especially telegraph poles, sleepers and the like, and it more particularly concerns impregnation by means of pressure other than normal. It is an object of my invention to improve this mode of impregnation with a view to saving time and impregnating material.

The impregnation of wood is effected mainly with the aid of mercury chloride, copper sulphate, zinc chloride, the fluorides of different metals, certain phenols, nitro-phenols or the salts of these compounds. As is well known to those skilled in the art, solutions of these substances can be introduced into the wood only with difficulty and in consequence thereof even several days will not suffice to impregnate more than the layers of wood adjoining the surface. In order to remedy this drawback it has been proposed to force the impregnating substance in by pneumatic means. To this end the wood is introduced in a closed impregnating vat, which as a rule has the form of an iron cylinder, and part of the air contained in the cylinder is then removed by pumping, whereupon the impregnating solution is forced into the cylinder under a pressure of several atmospheres, until the wood is thoroughly impregnated. This mode of proceeding, although being a distinct improvement of the practice formerly followed, requires a comparatively long time and involves the consumption of considerable quantities of impregnating substances.

I have now ascertained that the process of impregnating wood with the aid of reduced and increased pressure can be greatly improved both as regards time and consumption of chemicals, if, after the air has been removed from the impregnating vat, instead of a solution having the concentration required for full impregnation of the wood, a weaker solution is forced into the wood which, owing to its lower viscosity, readily penetrates into the interior of the wood. At the same time the cellular tissue of the wood is partly loosened, whereby the subsequent treatment with the stronger solution is greatly facilitated. Moreover, the weaker solution already suffices for preserving the interior of the wood so that it is not necessary to wait until the stronger solution which is subsequently introduced penetrates into the interior of the wood.

By arranging the impregnating vats in a suitable manner, for instance as described in my co-pending application for patent of the United States, filed of even date here-with, I also succeed in impregnating with the strong solution only that portion of the wood which is most exposed to destructive influences.

In the drawings affixed to this specification and forming part thereof the means for practising the novel process are illustrated diagrammatically by way of example.

Referring to the drawings, 5, 5 are the vats designed to receive the wood to be impregnated. In the drawing only a single pair of vats is shown, but I wish it to be understood that, as a rule, a battery of such vats arranged in pairs is required for the impregnation of larger masses of wood. After the vats have been filled with the wood, the covers are put on and the vats are partly evacuated by starting an air pump (not shown) connected with the piping 22. After the reduced pressure has been allowed to act during about 30 minutes the pipe 15 is opened which allows the impregnating solution to enter the lower part of the vats. This pipe is connected by means of the main 15' with the container 33 for the dilute solution containing for instance 350 g. mercury chloride in 300 liters water. After the valves 35 have been closed, the pipings 21 leading to the compressor (not shown) are opened. After compressed air has been allowed to act on the contents of the vats during about 30 minutes, the pipe 15' is opened again, allowing the liquid from the vats to be forced back into the container 33, which at the same time acts as a measuring vessel.

The main 15' is now closed and the air pump acting on pipe 22 is started anew. After 30-45 minutes the main 15'' is opened, which connects the impregnating vats with the second container 64 which contains the concentrated impregnating solution, which may for instance contain 650 g. mercury chloride in 300 l. water. This solution is now sucked into the impregnating vats, and in coming into contact with the wood thoroughly impregnates the layers of wood adjoining the surface. The action of the reduced pressure and of the dilute solution has already opened part of the cells of the wood and in consequence thereof the strong solution can now enter with some ease.

After the vats have been filled with the concentrated solution the air pump is brought to a stand-still and pipe 21 is opened, whereby the wood is placed under an increased pressure of about 3-7 atm., according to the density of the wood treated. Under the action of increased pressure, which is allowed to act thereon during about 30 minutes, the wood is thoroughly impregnated. At the end of this period pipe 27 is opened to relieve the vats of part of the pressure contained therein, the rest being utilized for expelling the liquid into the container 64 which also serves as a measuring vessel. The vats are then opened and the wood is removed.

I wish it to be understood that I do not desire to be limited to the exact materials, proportions and sequence of operations described for obvious modifications will occur to a person skilled in the art.

I claim:—

1. The method of impregnating wood comprising reducing the air pressure acting on the wood, allowing the dilute solution of an impregnating substance to enter the

wood while thus evacuated, thereafter once more reducing the pressure acting on the wood and then allowing a stronger solution of the impregnating substance to enter the wood.

2. The method of impregnating wood comprising reducing the air pressure acting on the wood, forcing into the wood a dilute solution of an impregnating substance at a pressure above the normal, removing the dilute solution surrounding the wood, evacuating the wood anew forcing into it a stronger solution of an impregnating substance under increased pressure and removing this stronger solution.

3. The method of impregnating wood comprising evacuating the wood, acting thereon with a mercury chloride solution containing 350 g. in 300 l. water, removing this solution, again reducing the air pressure acting on the wood and acting thereon with a solution containing 650 g. mercury chloride in 300 l. water.

In testimony whereof I affix my signature.

KARL BUBLA.